

## UNITED STATES PATENT OFFICE

2,253,308

## DESULPHURIZATION OF HYDROCARBONS

Raphael Rosen, Elizabeth, N. J., assignor to  
Standard Catalytic CompanyNo Drawing. Application May 5, 1937,  
Serial No. 140,836

6 Claims. (Cl. 196—28)

This invention relates to the process of desulphurization of a hydrocarbon containing organically combined sulphur by dehydrogenating organic compounds. It more particularly relates to desulphurization of a petroleum liquid.

According to the process of this invention, suitable hydrocarbons are dehydrogenated in a desulphurization operation to substantially increase the removal of the organically combined sulphur. It is within the scope of this invention to increase the efficiency and life of desulphurization catalysts by dehydrogenating organic compounds in the desulphurization operation. The preferred method is to add to a desulphurization operation suitable hydrocarbon compounds which will be dehydrogenated by means of dehydrogenation catalysts under the conditions of temperature and pressure of the operation. The hydrocarbons suitable for dehydrogenation may be added to increase the efficiency of any hydrocarbon desulphurization operation. However, the invention more particularly relates to their addition to the desulphurization of a virgin or cracked liquid petroleum hydrocarbon boiling between 100° F. and 700° F. and containing from 0.1% to 1% sulphur.

Any organic compound capable of being dehydrogenated under the conditions of the operation may be added, but it is preferred to use carbocyclic compounds particularly the hydroaromatics, examples of which are cyclohexane, methyl cyclohexane, ethyl cyclohexane, di and tetra hydronaphthalene. These preferred compounds for dehydrogenation may be used in a pure state but commercially they are found in complex mixtures containing all the varied structures of the desired compounds and other organic material not subject to dehydrogenation. In some cases at elevated temperatures, and especially in the presence of catalysts such as selenium or molybdenum or their compounds, other naphthenes such as cyclo pentane may be employed. However, it is preferred to employ hydroaromatic hydrocarbons and especially stocks containing at least 10% or preferably 20% to 30% or more of hydroaromatic hydrocarbons. Solvent extraction operations are one source of these complex mixtures in which selective solvents, as, for instance, liquid sulphur dioxide, acetonitrile, phenyl furfural, ortho anisidine, resorcinol diacetate, ethylene diacetate, tricresyl phosphate, triphenyl phosphate, aniline, acetone, propane and butane are employed.

If a selective solvent such as liquid sulphur dioxide is employed to extract a stock containing naphthenic and paraffinic compounds, the desired materials for dehydrogenating are found in the extract. Extraction products from certain stocks are preferred, as, for instance, stocks from

naphthenic crudes such as Sugarland or Quirquire or stocks from crudes containing quantities of naphthenic hydrocarbons such as Conroe, Colombian or West Texas. Another source of preferred material suitable for dehydrogenation is the raffinate secured by extracting the polymerization product of a thermal polymerization operation. In this operation usually propane and butane are cracked and polymerized at temperatures from 900° to 1050° F. and at pressures from 1000 to 2000 pounds per square inch. The product of this operation consists essentially of naphthenes and olefins and by extracting with a suitable solvent, preferably triethylene glycol, capable of selectively dissolving the olefin, a desirable raffinate high in naphthenic compounds results. The raffinates or extracts secured by the above methods may be used as such or may be hydrogenated to completely saturate with hydrogen, thereby increasing the hydrogen capable of being released per volume of added material under the conditions of the dehydrogenation operation.

Another source of a mixture containing desirable naphthenic and cyclic compounds is a product secured when destructively hydrogenating petroleum distillates. In this method either a straight run or cracked mineral oil is passed in vapor phase with hydrogen over suitable catalysts at pressures from 20 to 200 atmospheres or higher and at a temperature above 900° F. preferably within the temperature range of 930° F. to 1050° F. and the operating conditions and partial pressure of hydrogen so regulated to secure destructive hydrogenation without the formation of appreciable quantities of polymers or coky materials.

It is known that in a desulphurization operation, desulphurization catalysts of the classes of sulphides and oxides of tin, lead, iron, cobalt and molybdenum are effective. In addition, bauxite is also effective as a catalyst for desulphurization. However, for a certain type of sulphur compounds, particularly when the sulphur is organically combined, and especially when the sulphur is in the ring of the hydrocarbon compound, these catalysts even in the presence of hydrogen are inefficient and their life is relatively short.

It has been found that if suitable organic compounds as defined above, as, for example naphthenes and hydroaromatic hydrocarbons or mixtures containing these compounds are added to the materials being desulphurized in the presence of catalysts having desulphurization and dehydrogenation properties under conditions to produce dehydrogenation of the added material, the reduction in sulphur will be much greater and the life and activity of the catalyst will be increased.

Any catalyst producing dehydrogenation of the added cyclic or naphthenic compounds is satisfactory. The catalysts employed for desulphurization will also usually be satisfactory as dehydrogenation catalysts under the conditions of the process. If these desulphurization catalysts are not suitable, satisfactory dehydrogenation catalysts may be added. The preferred catalysts for dehydrogenation are oxides and sulphides of the metals of Group VI of the periodic table and oxides and sulphides of zinc, aluminum, vanadium and palladium. The salts of these metals treated substantially in a manner as given in Example 1 are also satisfactory. The catalytic metals may also be satisfactory when contained in the acid radical of a salt, as, for example, chromium in lead chromate. The operation may be carried out under any conditions which produce dehydrogenation of the added materials, as for instance at temperatures from about 300° to 1200° F. However, the preferred conditions are temperatures from about 700° F. to 1100° F. or higher and at pressures varying from 12 to 100 pounds per square inch absolute.

The following examples will serve to illustrate the invention:

#### Example 1

Benzine was passed over a catalyst of lead chromate, zinc sulphate and magnesium oxide, prepared in the following manner: commercial magnesite (6 to 10 mesh) was burned at from 1000° F. to 2000° F. for one hour. 100 grams of the burned magnesite was then treated with 200 ccs. of 5% potassium dichromate solution for one-half hour at the boiling point of the solution, then filtered and dried at 572° F. The dried catalyst was then treated with 200 ccs. of 7½% lead acetate solution for one-half hour at the boiling point of the solution; then filtered, thoroughly washed and dried at 572° F. 75 grams of this lead chromate on burned magnesite was then treated with 150 ccs. of 25% zinc sulphate solution at the boiling point of the solution, filtered, first dried at 572° F. and finally at 932° F.

In Test A, the benzine contained 0.311% sulphur and the results as shown are the average of the 7 samples run. In Test B, the benzine solution contained 75% benzine, 25% tetra hydro naphthalene and 0.465% sulphur, and the results as shown are averages of the four samples run. Fresh catalysts were used for each test.

The temperature and pressure conditions of the benzine desulphurization operation with results secured were as follows:

|             | Vol./liq./hr.<br>per vol. of<br>cat. | Temp.,<br>°F. | Pressure       | Per cent<br>sulphur<br>removed |
|-------------|--------------------------------------|---------------|----------------|--------------------------------|
| Test A----- | .74                                  | 950-1000      | Atmospheric... | 21.6                           |
| Test B----- | .97                                  | 950-1000      | do-----        | 41.7                           |

In Test B, it was observed that hydrogen sulphide was evolved which was not observed in Test A. The above shows that in Test B, in which a substance suitable for dehydrogenation was added, even with a higher volume of liquid per volume of catalyst, the per cent reduction in sulphur was about doubled.

10

#### Example 2

A benzine solution containing 0.224% sulphur as thiophene and 25% tetra hydro naphthalene in Test A was passed over a catalyst of lead chromate, zinc sulphate and magnesium oxide, while in Test B a benzine solution containing 0.228% sulphur as thiophene was passed over an identical fresh catalyst with the following results:

|             | Vol./liq./hr.<br>per vol. of<br>cat. | Temp.,<br>°F. | Pressure       | Per cent<br>sulphur<br>removed |
|-------------|--------------------------------------|---------------|----------------|--------------------------------|
| Test B----- | .19                                  | 950-1000      | Atmospheric... | 13.7                           |
| Test A----- | .27                                  | 950-1000      | do-----        | 42.0                           |

The above example shows that with a higher volume of liquid per volume of catalyst, the sulphur reduction secured with the added dehydrogenating compound was over three times the reduction secured when not adding this type of compound.

35

#### Example 3

A California cracked distillate cut to 400 end point before cracking having an initial boiling point of 120° F. and a final boiling point of 412° F. with 90% off at 347° F. and a gravity of 52.9 A. P. I. with an aniline point of 103 containing 0.98% sulphur was passed over a dehydrogenating catalyst prepared from lead chromate, zinc sulphate and magnesium oxide both with and without the addition of a naphthenic hydrocarbon with the following results:

|                                                      | Vol./liq./hr.<br>per vol. of<br>cat. | Temp.,<br>°F. | Pressure       | Per cent<br>sulphur<br>removed |
|------------------------------------------------------|--------------------------------------|---------------|----------------|--------------------------------|
| Test A—a California distillate.                      | .143                                 | 950-1000      | Atmospheric... | 18.4                           |
| Test B—a California distillate plus 25% cyclohexane. | .143                                 | 950-1000      | do-----        | 26.7                           |

60

#### Example 4

The following data demonstrates clearly the marked advantage and improvements secured by the present process over the process of treating with hydrogen gas.

65

| Test<br>run,<br>hours | Catalyst                 | Reaction<br>temperature,<br>°F. | Pressure       | Vol. feed<br>per hr.<br>per vol.<br>catalyst | Hydro-<br>carbon<br>vapor per<br>vol. H <sub>2</sub> in<br>feed | Sulphur, per cent |         |         |
|-----------------------|--------------------------|---------------------------------|----------------|----------------------------------------------|-----------------------------------------------------------------|-------------------|---------|---------|
|                       |                          |                                 |                |                                              |                                                                 | Original          | Treated | Removed |
| 3-----                | Molybdenum sulphide----- | 842                             | Atmospheric... | 1-12                                         | 1-1-----                                                        | .214              | .187    | .22     |
| 32-----               | do-----                  | 842                             | do-----        | 1-6                                          | 10% tetralin                                                    | .221              | .159    | .28     |

Thus, from the above it may be seen that the present process secured approximately 25% greater removal of sulphur at the same temperature and at atmospheric pressure with half the catalytic volume. Furthermore, even though neither test was run to determine the catalytic life, it is extremely significant that the data indicating the marked improvement of the present process was secured by comparing a run of 32 hours to a short run of three hours during which in this latter case the activity of the catalyst was at a maximum.

The foregoing examples are merely illustrative. Temperatures and pressures and any particular method of handling may be varied within the scope of the invention, but the invention is not to be limited by any theory of operation, but only by the following claims in which it is desired to claim all novelty insofar as the prior art permits.

I claim:

1. A process of desulphurizing a normally liquid hydrocarbon mixture boiling within the gasoline range and containing organically combined sulphur which comprises adding to said hydrocarbon mixture a hydrocarbon composition containing at least one carbocyclic hydrocarbon wherein in two hydrogen atoms are attached to each of at least two nuclear carbon atoms, the carbocyclic hydrocarbon content of said hydrocarbon composition amounting to at least 10%, passing the resultant hydrocarbon mixture in contact with a dehydrogenation catalyst under dehydrogenating conditions at substantially atmospheric pressure and removing the hydrogen sulphide from the reacted mixture, the reaction being carried out in the absence of added free hydrogen.

2. A process which comprises adding tetrahydronaphthalene to a benzine containing organically combined sulphur and contacting the mixture with a dehydrogenation catalyst at the rate of about .97 volume of benzine mixture measured as liquid per hour per volume of catalyst at a temperature between about 950 and about 1000° F. at substantially atmospheric pressure and removing hydrogen sulphide from the product, the reaction being carried out in the absence of added free hydrogen.

3. A process which comprises adding cyclohexane to a cracked petroleum distillate having an initial boiling point of about 120° F., a final boiling point of about 412° F., an A. P. I. gravity of about 52.9, an aniline point of about 103 and containing about 0.98% of organically bound sulphur, contacting said mixture with a dehydrogenation catalyst prepared from lead chromate, zinc sulphate and magnesium oxide at a throughput of about .143 volume of mixture measured as liquid per hour per volume of dehydrogenation catalyst at a temperature between about 950 and about 1000° F. and removing the sulphur-containing vapors from the product.
4. A process for desulphurization of a petroleum hydrocarbon containing organically combined sulphur comprising adding to a petroleum hydrocarbon boiling between 100 and 700° F. and containing from about .1 to 1% sulphur, at least 10% of a hydroaromatic hydrocarbon, passing the mixture over a dehydrogenation catalyst at a temperature in the range of from about 300° F. to about 1200° F. and under a substantially atmospheric pressure and separating hydrogen sulphide from the resulting products, the reaction being carried out in the absence of added free hydrogen.
5. A process in accordance with claim 4 in which said hydrocarbon is a cracked petroleum distillate containing from about 0.1% to about 1% sulphur.
6. A process for desulphurizing a cracked hydrocarbon distillate containing organically combined sulphur, comprising adding to a cracked distillate boiling in the range from about 100 to about 700° F. at least 10% of a hydroaromatic concentrate secured by solvent extraction of hydrocarbon fractions with suitable extracting agents selected from the class of solvents having a preferential selectivity for the more aromatic type hydrocarbons, passing said mixture in contact with dehydrogenation catalysts at temperatures between about 300° F. and about 1200° F. and under substantially atmospheric pressure and separating the hydrogen sulphide formed, the reaction being carried out in the absence of added free hydrogen.

RAPHAEL ROSEN.